

May 11, 1926.

1,584,689

H. E. BAKKEN

# PROCESS AND APPARATUS FOR VOLATILIZING METAL

Filed April 27, 1921



H. E. Bakken

By John Boyle Jr.  
My

## UNITED STATES PATENT OFFICE.

HERMAN E. BAKKEN, OF NIAGARA FALLS, NEW YORK, ASSIGNOR TO AMERICAN MAGNESIUM CORPORATION, OF NIAGARA FALLS, NEW YORK, A CORPORATION OF NEW YORK.

## PROCESS AND APPARATUS FOR VOLATILIZING METAL.

Application filed April 27, 1921. Serial No. 464,823.

My invention relates to a process and apparatus for volatilizing metal from fused metalliferous material and particularly to the electrolytic production of magnesium from its fused salts, and one of the objects of the invention is to electrolytically decompose the metallic salts and collect the metal therefrom ultimately in the form of a pure distillate. Altho particularly adapted for magnesium, the invention is equally applicable to the other metals which have similar characteristics.

The application of my invention is illustrated herein, in connection with the oxide process of producing magnesium as disclosed in the patents to Seward 1,210,449, and 1,310,450 granted July 22, 1919. In those patents, there is disclosed a method of producing magnesium, comprising the electrolysis of a molten bath of mixed fluorids, including magnesium fluorid, and magnesium oxide. The bath is of such a specific gravity that it will support on its surface a crust of magnesium oxide and any separated metal will rise to the top of the bath and collect beneath the said crust. The metal is intermittently removed by punching a hole in the crust and ladling it out by hand. The disadvantages of this method are that the metal contains undesirable impurities such as silicon and to secure pure metal must be refined by a separate operation; also the temperature at which the bath is operated may be so high as to cause loss of metal by evaporation.

In the drawing Fig. 1 is a sectional elevation of the apparatus used in carrying out my invention, and

Fig. 2 is a section on the line 2—2 of Fig. 1.

Referring to the drawing, 10 is a tank for holding the fused bath material and having anodes 11 along the median line thereof and cathodes 12 on both sides of the anodes. The metallic magnesium separates at the cathodes and being lighter than the bath material has a tendency to rise to the top of the bath.

Suspended directly over each cathode is an elongated bell or box 13 only one of which is shown, which may be completely submerged in the molten bath. Rising from its centre point is a conduit 14 which extends upward a suitable distance. At its upper

end the conduit 14 is connected to a down coming conduit 15, the latter being connected at its lower end with a suitable condenser 16. Both of the conduits 14 and 15 may be covered with insulation 23 for preventing loss of heat by radiation. Adjacent the condenser 16 is a container 17 for holding a metal mold 18. The condenser 16 and the container 17 are connected by a pipe 19 and also by a pipe line 20 containing valves 21. The pipe line 20 is adapted to be connected at 22 with a vacuum pump for creating a vacuum in the entire system. For maintaining the desired temperature of this system any suitable means may be used, but I prefer to use electrical heating means.

The operation of my invention is as follows: When a vacuum is established in the conduit 14, the result will be that the bath material will rise therein. The height of the column of bath will depend on the amount of the vacuum and the specific gravity of the bath material. Any globules of metal separated at the cathode, on account of their specific gravity being lower than the bath material, will rise to the surface and collect under the bell 13 and from there rise thru the bath material in the conduit 14. Due to the decreased pressure on the column of bath material, the boiling point of the molten metal, within the influence of the decreased pressure, will be lowered. The metal which has separated in a liquid form at the temperature of the bath and at atmospheric pressure, will, by the time it has reached the top of the column, be transformed into metallic vapor, which will pass over and be condensed in the condenser 16. The metal in the condenser 16 will remain liquid but that in the pipe 19 will solidify. By intermittently thawing out the pipe 19, which may be heated by any suitable means, then closing the vacuum line to the condenser 16 and opening it up to the container 17, the collected metal may be transferred from time to time into the mold 18. This arrangement allows the distillation to proceed continuously while the transference and removal of the metal is intermittent.

While I have particularly described my invention in connection with the electrolytic production of magnesium from its fused salts, and as an exemplification, a process in which magnesium rises to the surface

of the molten bath, it is not intended to so limit its use. For instance there may be other metalliferous material than that specified to which the invention might be applied, and the metal may be plated out on to a molten cathode at the bottom of the bath and subsequently separated therefrom by distillation. While I have illustrated and described the preferred embodiment of the invention, it will be understood that I reserve the right to all changes properly falling within the scope and spirit of the appended claims.

I claim:

- 15 1. The process of reducing magnesium from its fused salts comprising subjecting the fused salts to electrolysis and simultaneously volatilizing the separated magnesium at less than atmospheric pressure.
- 20 2. The process of reducing magnesium from its compounds comprising subjecting a bath of the fused compounds to electrolysis, the specific gravity of the bath being sufficiently high to cause the separated magnesium to rise to the surface of the bath, reducing the pressure to promote volatilization of and thereafter condensing the metallic vapor.
- 25 3. The process of reducing magnesium from its compounds comprising subjecting fused metalliferous material to electrolysis, a portion of fused material being at atmospheric pressure and another portion being at less than atmospheric pressure.
- 30 35 4. The process of reducing magnesium from its compounds comprising subjecting fused metalliferous material to electrolysis and causing a portion of fused magnesium containing material to take a position where
- 40 45 it is subjected to less pressure than the main body thereof and maintaining such temperatures and pressures so that the separated metal will remain liquid in the main body thereof and vaporize in the said portion.
- 50 55 5. The process of reducing magnesium from its compounds comprising subjecting fused metalliferous material to electrolysis, causing a portion of fused magnesium containing material to take a position where it may be subjected to less pressure than the main body thereof, maintaining such a temperature in the main body so that the separated metal will remain liquid therein, maintaining substantially the same temperature in the said portion as in the main body, but reducing the pressure thereon in order to promote volatilization of the metal therein.
- 60 65 6. A process of reducing magnesium from its compounds comprising subjecting fused metalliferous material to electrolysis, said material comprising magnesium oxide and magnesium fluorid, and causing a portion of fused magnesium containing mate-

rial to take a position where it is subjected to less pressure than the main body thereof and maintaining such temperature and pressure that the separated metal will remain liquid in the main body thereof and 70 vaporize in the said portion.

7. The process of reducing magnesium from its compounds comprising subjecting fused metalliferous material to electrolysis, causing a portion of the fused magnesium containing material to take a position where it is subjected to less pressure than the main body thereof, the specific gravity of the bath being sufficiently high to cause the separated magnesium to rise therein and maintaining such temperature and pressure that the separated metal will remain liquid in the main body thereof and vaporize in the said portion.

8. The process of volatilizing metal from fused metalliferous material comprising subjecting a portion of the said material to such temperature and pressure so that the contained metal will not substantially volatilize and subjecting another portion to such temperature and pressure, so that the contained metal will volatilize.

9. The process of volatilizing metal from fused metalliferous material comprising causing a portion of fused material to take a position away from the main body, subjecting the main body of the material to atmospheric pressure and to such temperature so that it will not substantially volatilize and subjecting the said portion to less than atmospheric pressure and such temperature, so that the contained metal will volatilize.

10. An apparatus of the character described, comprising a receptacle for holding fused metalliferous material, a conduit combined with the receptacle and adapted to contain fused material, a condenser for metallic vapor, means for maintaining a vacuum in the conduit to cause fused material to rise therein and metal to volatilize, the length of the conduit being greater than the height of the column of fused material therein.

11. An apparatus of the character described comprising a receptacle for holding fused metalliferous material, a conduit combined with the receptacle and adapted to contain fused material, means for maintaining a vacuum in the conduit to cause the metalliferous material to rise therein and the contained metal to volatilize.

12. An apparatus for the electrolytic reduction and distillation of metals, comprising a tank for holding fused metalliferous materials, a conduit combined with the tank and adapted to contain fused material, means for controlling the temperature of the fused material in the conduit, and a condenser for metallic vapor connected to

the conduit and means for maintaining a vacuum in the conduit to cause fused material to rise therein and the contained metal to volatilize.

5 13. In combination with a furnace for volatilizing metal, a condenser, a mold adjacent thereto, means for conducting the metal from the condenser to the mold and means for preventing contact of the air 10 with the metal.

14. A process for the production of metals, comprising electrolyzing a molten bath containing a compound of the metal desired, and withdrawing the metallic prod-

ucts of the electrolysis in vapor form and 15 at a pressure less than atmospheric.

15. A process for making magnesium, comprising electrolyzing a magnesium salt at a temperature of at least 650° C., approximately, and under a pressure low 20 enough to permit vaporization of the magnesium produced, withdrawing the magnesium vapor apart from the anodic products of the electrolysis, and condensing the magnesium vapor so withdrawn. 25

In testimony whereof I affix my signature.

HERMAN E. BAKKEN.